

## UNITED STATES PATENT OFFICE.

WILLIAM F. DOERFLINGER, OF WEST NEW BRIGHTON, NEW YORK.

## ELECTRICAL INSULATION.

No Drawing.

Application filed June 22, 1928. Serial No. 287,652.

This invention relates particularly to dielectric substances and to electrical devices, such as transformers, oil switches and the like, in which conducting bodies differing in electrical potential are separated by a dielectric liquid.

It is desirable that the liquid insulating medium or dielectric, in such devices, combine in high degree high dielectric strength, freedom from moisture, acid and alkali etc., low evaporation loss for prolonged periods, high flash point, high burning point, small affinity for water, and small tendency to form carbonaceous deposits or otherwise decompose. A considerable fluidity (or low viscosity) is also often of importance.

Various materials, such as hydrocarbon oils, rosin oils, vegetable oils, etc., have been used for this purpose.

20 I have found that tricresyl phosphate is more suitable as a dielectric liquid than most substances which have been proposed for this purpose.

Tricresyl phosphate is an odorless, colorless liquid, neutral in character, non-hygroscopic, and immiscible with water, has a high flash point and is substantially non-volatile and non-burnable. It is freely fluid and has a high dielectric strength. It is very 30 stable.

I have found the dielectric strength tested between one inch disc electrodes spaced one-tenth inch apart in accordance with A. S. T. M. Specification D 117-24 entitled "Standard 35 method of testing transformer and switch oils" using a transformer rated at 125 K. V., 25 K. V. A, supplied with current at 120 volts 60 cycles is about 13,700 volts at puncture,

using ordinary good commercial material without special drying or other treatment. 40

The flash point is about 460° F. and the burning point about 705° F. It can be made to burn only with extreme difficulty.

45 The high burning point of tricresyl phosphate is of great importance in closed transformers of large size; also its fluidity, which is rather remarkable for a substantially non-volatile liquid. This enables it to convey away heat generated in the transformer very efficiently, and readily self-heat in case of a 50 discharge.

55 My invention is not concerned with the electrical construction of transformers, switches etc. In practicing it I merely use tricresyl phosphate in place of the hydrocarbon oils etc. which are at present employed in apparatus of this type, such as oil insulated transformers.

What I claim is:—

1. An electrical device comprising conductors adapted in use to have different electrical potential, separated by a dielectric comprising tricresyl phosphate. 60

2. An electrical device using liquid insulation including a dielectric comprising tricresyl phosphate. 65

3. An electrical device using insulation consisting of tricresyl phosphate, substantially as and for the purpose described.

4. An electric device using insulation consisting of liquid tricresyl phosphate. 70

5. An electrical device comprising conductors separated by liquid tricresyl phosphate.

This specification signed this 20th day of June, 1928.

WILLIAM F. DOERFLINGER.